

1

**3,399,079  
ANTISTATIC FIBER BLEND**

Seth Owens Harris, Danbury, Conn., and Charles Alexander Ball, Mount Vernon, N.Y., assignors to American Cyanamid Company, Stamford, Conn., a corporation of Maine  
No Drawing. Filed Sept. 25, 1964, Ser. No. 399,396  
5 Claims. (Cl. 117—138.8)

**ABSTRACT OF THE DISCLOSURE**

A blend of hydrophobic synthetic fibers having improved antistatic properties and improved processability through textile machines consisting essentially of a major proportion comprising from about 55% to about 90% of the fibers in the blend having applied thereto a durable friction-reducing antistatic agent and a minor proportion comprising from about 10% to about 45% of the fibers in the blend having applied thereto a friction-increasing agent.

This invention relates to synthetic fibers which have improved antistatic properties and improved processability through textile machines. More particularly, these two desirable characteristic of synthetic fibers, are achieved through the use of the present invention wherein a major proportion of the fibers in a blend of such fibers have incorporated therein a durable antistatic agent while the remaining minor proportion of the fibers in such blend have incorporated therein a friction-increasing agent, which, preferably, is a nondurable antistatic agent.

The difficulties arising from the generation and accumulation of static electricity in synthetic fibers, due to their hydrophobic nature, are well known. These difficulties arise during the use of end products made from such fibers, and, to an even greater extent, during textile processing and manufacturing operations to make such end products.

In order to overcome these difficulties, it has been proposed to apply durable antistatic agents to these fibers or to a minor proportion of such fibers in a blend with a major proportion of untreated fibers.

Unfortunately, such techniques have resulted in greatly increased difficulties in processing the yarns through the textile machinery necessary to convert staple fibers into threads (as compared with naturally antistatic hydrophilic fibers such as cotton and wool). However, these durable antistatic agents do produce textile fabrics which have a softer hand than would be achieved with the same fibers which are untreated.

In accordance with the present invention, it has been found that greatly improved textile processability of these hydrophobic fibers can be achieved while producing satisfactory antistatic properties by blending a major proportion of fibers having incorporated therein a durable antistatic agent with a minor proportion of fibers having incorporated therein a friction-increasing agent, which preferably is a nondurable antistatic agent.

The need for the friction-increasing agent became apparent when we discovered that the cause of poor processability of the synthetic fibers treated with a durable anti-

2

static agent resulted from a lowering of the frictional characteristics of such yarns.

However, it was also discovered that the textile fabrics made from yarns processed in accordance with our invention had a relatively harsh hand unless the friction-increasing agent was nondurable (i.e., could be readily removed from the fabrics by scouring, washing, etc.). Accordingly, our invention therefore contemplates that the friction-increasing agent preferably be a nondurable agent when it is desired to produce fabrics having a relatively soft hand.

Also, since the tendency of hydrophobic fibers to build up static charges is much greater during the conditions of textile processing, particularly those encountered in picking and carding, then it is during conditions of consumer use of the textile products, it is important that the fibers have a higher degree of antistatic properties during textile processing. Accordingly, the friction-increasing agent should also possess antistatic properties so as to provide the higher degree of protection necessary during the textile processing operations.

Illustrative of hydrophobic synthetic fibers which are of particular interest in the practice of our invention are those fibers prepared from vinyl polymers, for example, acrylic fibers, polypropylene fibers, polyvinyl chloride fibers, and the like, and fibers prepared from polymers of polyesters, polyacetics, polyurethanes, and polyamides.

Any of the many durable antistatic agents commonly known may be used on the major proportion of the hydrophobic fibers. Illustrative of these durable antistatic agents are those formed from polyethylene glycol, such as the condensation products of polyethylene glycol diamine and polyethylene glycol dihalide of which Aston 108, Aston 123, and Aston LT sold by Onyx Chemical Corporation, and Stanax and Stanax 1166 sold by Standard Chemical Products, Inc., are commercially available examples. These compounds may be cured with polyepoxides after application to the fibers to produce a durable antistatic finish therein and thereon by such processes as taught in Anthes U.S. Patent 2,982,751, issued May 2, 1961, which also lists other compounds of this type useful in the practice of our invention. Similarly, these compounds may be cured with dihalides. Also useful are other compounds sold for use as durable antistatic agents such as Zerostat P (polyoxyethylene diepoxide, cross-linked with a diamine) sold by Ciba Chemical and Dye Co. and Aerotex Antistatic No. 6 (polyoxyethylene amine, cross-linked with cyanuric chloride) sold by American Cyanamid Company.

These durable antistatic agents may be applied to the fibers at any stage of processing in any of the conventional ways. It is important only that the durable antistatic agent be applied to the fibers prior to blending them with other fibers which have been treated with a friction-increasing agent, which blending occurs prior to formation of the fibers into threads. Preferably the durable antistatic agent is incorporated on the fibers in an amount between about 0.25% and about 2.0% based on the weight of fibers so treated. It is important that the fibers treated with the durable antistatic agent constitute a major proportion of the fibers in the blend, preferably from 55% to 90% thereof.

Any of a large number of friction-increasing agents commonly known can be used on the minor proportion

of the hydrophobic fibers. Illustrative of these friction-increasing agents are the following:

| Name                         | Description                                      | Sold By                        |
|------------------------------|--------------------------------------------------|--------------------------------|
| Perimolite                   | Solubilized alkyl resin                          | Arkansas Co., Inc.             |
| Aerotex Resin 700            | Urea-formaldehyde condensate                     | American Cyanamid Co.          |
| Aerotex Resin 803            | Modified urea-formaldehyde condensate            | Do.                            |
| Iberantslip                  | Solubilized protein                              | A. Harrison & Co., Inc.        |
| Kolina Adhesive              | Modified vinylpyrrolidone resin                  | Antara Chemical Co.            |
| Atlas G-750                  | Sodium sorbital borate                           | Atlas Chemical Industry, Inc.  |
| Atlas G-3300                 | Alkylamine alkane sulfonate                      | Do.                            |
| Non-slip Finish No. 22       | Water-soluble modified resin                     | Apex Chemical Co., Inc.        |
| Beratex No. 510              | Modified alkylarylsulfonate                      | Berkshire Color & Chemical Co. |
| Arogum                       | Protein blend                                    | Arol Chemical Product Co.      |
| Larnol 60-98                 | Polyvinyl alcohol                                | Borden Chemical Co.            |
| Estralok A                   | H <sub>2</sub> O soluble polymerized resin ester | Crown Chemical Corp.           |
| Melltone SCR                 | Polyoxyethylene ester composition                | Do.                            |
| Lubritone SA                 | Emulsified lubricants                            | Chas. S. Tanner Co.            |
| Conco Non-slip Special A & B | Viscid water-soluble resin                       | Continental Chemical Co.       |
| Lureen Special               | Fatty based derivative w/bonding agents          | George A. Gautston Co.         |
| Krinkle Finish               | Emulsified fatty esters                          | Grestebo Dyes & Chemical, Inc. |
| Syton DS                     | Colloidal silica                                 | Monsanto Chemical Co.          |
| Lenoscroop-600               | Modified fatty ester emulsion                    | Lenox Chemical Co.             |
| Cachalot 0-21                | Oleyl alcohol                                    | M. Michel & Co.                |
| Atco Bindtex R               | Water-soluble resin                              | Metro-Atlantic, Inc.           |
| Prosoxet CR                  | Blended organic acids                            | Quaker Chemical Corp.          |
| Standafin 92                 | Water-soluble thermoplastic resin                | Standard Chemical Product Inc. |

In the preferred embodiments of our invention, the friction-increasing agent also serves as an antistatic which is nondurable (i.e., easily removed from the fibers in the finished product by washing or scouring). Illustrative of these non-durable friction-increasing antistatic agents are the following:

| Name                    | Description                                                  | Sold By                             |
|-------------------------|--------------------------------------------------------------|-------------------------------------|
| Aerotex Antistatic CSN. | Cationic organic compound.                                   | American Cyanamid Co.               |
| Pergal TW               | Alkyl poly(ethyleneoxy) glycol amine.                        | General Aniline & Film Corp.        |
| Atlas G-263             | N-cetyl-N-ethylmorpholinium ethosulfate.                     | Atlas Chemical Inc.                 |
| Atlas G-3780A           | Polyoxyethylene amine condensate.                            | Do.                                 |
| Chemstat ON             | Blend of cationic agents                                     | Chemical Corp. of America           |
| Zerostat C              | Quaternary ammonium compound.                                | Ciba Chemical & Dye Co.             |
| Lekrostat B, GV         | Heterocyclic amine.                                          | Dexter Chemical Corp.               |
| Lekrostat C             | Fatty amine salts                                            | Do.                                 |
| Aquazine 88             | Fatty hydrazinium chloride                                   | Moretex Chemical Products Inc.      |
| Orco-Antistatic 83L     | Cationic compound.                                           | Organic Chemical Corp.              |
| Parastat S              | Polyoxyethylene alkylamine.                                  | Trylon Chemical Corp.               |
| Borne-stat              | Polyalkylaryl sulfonate.                                     | Borne Chemical Co.                  |
| Dowfax 2A1              | Dodecyldiphenyloxide disulfonic acid.                        | Dow Chemical Co.                    |
| Emkastat K              | Sulfonated aliphatic compound.                               | Emkay Chemical Co.                  |
| Seyco Stat-96           | Blend of fatty esters and polyoxyethylene fatty derivatives. | Seydel-Wodley & Co.                 |
| Zelac NE                | Alcohol phosphate composition.                               | Du Pont.                            |
| Cirrasol GM             | Polyglycol ester.                                            | Arnold, Hoffman & Co.               |
| Lubrol WX               | Fatty-alcohol ethylene oxide condensate.                     | Do.                                 |
| Carbowax                | Polyethylene glycol.                                         | Union Carbide Chemical Co.          |
| Sorbinox L-20           | Polyoxyethylene sorbitan monolaurate.                        | Trylon Chemical Corp.               |
| Paralube 20             | do.                                                          | Do.                                 |
| Textiline 3645          | Nonionic esters and hydrocarbons.                            | Sonneborn Chemical & Refining Corp. |
| Sonostat-60             | Nonionic derivative.                                         | Do.                                 |
| Syn-stat 400            | Polyethylene glycol derivatives.                             | Syn-Chemical Corp.                  |
| Syn-stat BH             | Complex phosphated alcohol.                                  | Do.                                 |

| Name               | Description                                      | Sold By                           |
|--------------------|--------------------------------------------------|-----------------------------------|
| Syn-stat D-20      | Polyethylene glycol derivatives.                 | Syn-Chemical Corp.                |
| Stantex 819        | Blend of fatty and synthetic lubricants.         | Standard Chemical Products.       |
| 5 Elosol SG        | Ethylenoxide condensate.                         | Do.                               |
| Elosol V           | Amphoteric compound.                             | Sandoz, Inc.                      |
| Lubrofin           | Polyoxyethylene esters.                          | Richmond Oil, Soap & Chemical Co. |
| Nopcostat AS-40    | Fatty amide.                                     | Nopco Chemical Co.                |
| Nopcostat 2152X    | Fatty ester.                                     | Do.                               |
| 10 Nopcostat LV-40 | Fatty amide and fatty ester.                     | Do.                               |
| Vinset             | Fatty acid ethylene oxide condensate.            | Metro-Atlantic, Inc.              |
| Lenostat Plus      | Blend of nonionic esters.                        | Lenox Chemical Co.                |
| Lenoscroop 125     | Modified fatty ester emulsion.                   | Do.                               |
| 15 Conditionol     | Blend of humectant agents w/amine condensates.   | Maker Color & Chemical Co.        |
| Conditionol W      | Mixture of sulfonated oils, resins and alcohols. | Bryant Chemical Co.               |
| 20 Tween 20        | Polyoxyethylene sorbitan monolaurate.            | Atlas Chemical Industries, Inc.   |
| Myrl 45            | Polyoxyethylene stearate.                        | Do.                               |

25 These friction-increasing agents may be applied to the fibers at any stage of processing in any of the conventional ways. It is important only that they be applied to the fibers prior to blending them with other fibers which have been treated with a durable antistatic agent, which blending occurs prior to formation of the fibers into threads. Preferably the friction-increasing agent is incorporated on the fibers so treated in an amount sufficient to increase the frictional characteristics of the blend of fibers to a level comparable to those fibers for which the textile processing equipment was designed, as in the cotton system, the woolen system, and the worsted system. Usually this can be achieved with the use of an amount of friction-increasing agent between about 0.25% 30 and 1.0% based on the weight of fibers so treated. It is important that the fibers treated with the friction-increasing agent constitute a minor proportion, preferably from 10% to 45%, of the fibers in the blend, particularly when such agent is nondurable.

35 The following examples will serve to illustrate a particular embodiment of our invention and some of the advantages thereof. In each of these examples, the fibers used were acrylic fibers of a copolymer of acrylonitrile and methylmethacrylate prepared by wet-spinning from an aqueous sodium thiocyanate solution thereof.

#### 50 Example 1

55 Crimped acrylic fibers were padded in a trough with a formulation containing Aston 108 (a condensation product of polyethylene glycol diamine and polyethylene glycol dihalide), cut into 2" staple, wet opened, dried at about 60° C. for about nine minutes, and then cured with a polyepoxide as taught in Anthes U.S. Patent 2,982,751, issued May 2, 1961, for about nine minutes at about 60 114° C. to form a product identified as Fiber A which contained about 0.6% durable antistatic agent based on weight of fiber.

65 Other acrylic fibers were padded with Nopco LV-40 finish (a mixture of fatty amides and fatty esters), crimped, cut into 2" staple, wet opened, and dried at about 60° C. for about nine minutes to form a product identified as Fiber B which contained about 0.5% non-durable friction-increasing antistatic agent based on weight of fiber.

70 A blend was prepared containing 65% Fiber A and 35% Fiber B by introducing the dry fibers in the proper proportions into a wet opener and then passing the mixture through a dry opener. The resulting blend was readily processable through the cotton system (which includes 75 picker, card, draw frame, roving frame, and spinning

frame) without difficulty. Woven and knitted products from threads so made from this blend of fibers exhibited a very soft hand after washing and scouring to remove the nondurable finish while still exhibiting satisfactory resistance to the accumulation of static charges.

#### Example 2

In a manner similar to that of Example 1, other blends were prepared in which a major proportion of the fibers were treated with a durable antistatic agent and a minor proportion of the fibers were treated with a friction-increasing agent. The durable antistatic agent and the friction-increasing agent were applied to their respective lots of fibers utilizing the general procedures of Example 1. These blends, detailed in the following table, all produced fiber blends having the characteristics indicated in the table. It will be noted that in all cases where the percent of fibers treated with the durable antistatic agent was equal to or greater than 55%, the processability on

at all on textile equipment. These fibers were not blended with any other fibers.

|                           | Antistatic Agent | Percent Finish on Fiber   | Processability | Antistatic Rating |
|---------------------------|------------------|---------------------------|----------------|-------------------|
| 5 Stanax                  | 0.25             | Poor                      | Fair.          |                   |
|                           | 0.50             | Very poor                 | Good.          |                   |
|                           | 0.75             | Not processable           |                |                   |
| 10 Stanax 1166            | 1.00             | do                        |                |                   |
|                           | 1.00             | Very poor                 | Do.            |                   |
|                           | 1.00             | Not processable           |                |                   |
| 15 Aston 108              | 0.25             | Poor                      | Fair-Poor.     |                   |
|                           | 0.5              | Very poor                 | Good.          |                   |
|                           | 0.75             | Not processable           |                |                   |
|                           | 1.0              | do                        |                |                   |
|                           | 1.75             | do                        |                |                   |
| Aston 123                 | 0.25             | Poor-very poor            | Fair.          |                   |
|                           | 0.5              | Very poor-not processable |                |                   |
| Aerotex Antistatic No. 6. | 0.75             | Not processable           |                |                   |
|                           | 0.5              | do                        |                |                   |
|                           | 1.0              | do                        |                |                   |
|                           | 2.0              | do                        |                |                   |

| Durable antistatic agent (D-A) | Percent D-A on fiber | Percent D-A treated fiber in blend | Friction-increasing agent (F-I) | Percent F-I on fiber | Percent F-I treated fiber in blend | Processability on textile equipment | Antistatic rating after 10 machine washes |
|--------------------------------|----------------------|------------------------------------|---------------------------------|----------------------|------------------------------------|-------------------------------------|-------------------------------------------|
| Stanax                         | 0.25                 | 80                                 | Nopostat LV-40                  | 0.5                  | 20                                 | V. good                             | Fair-good.                                |
|                                | 0.50                 | 65                                 | do                              | 0.7                  | 35                                 | do                                  | Good.                                     |
|                                | 0.75                 | 75                                 | do                              | 0.7                  | 75                                 | do                                  | Do.                                       |
|                                | 1.0                  | 65                                 | do                              | 0.5                  | 35                                 | Good                                | Do.                                       |
|                                | 1.0                  | 25                                 | Atlas G-3300                    | 0.5                  | 75                                 | V. poor                             | Poor.                                     |
|                                | 2.0                  | 55                                 | Nopostat LV-40                  | 0.5                  | 45                                 | Good                                | Good-fair.                                |
| Stanax 1166                    | 0.25                 | 75                                 | do                              | 0.4                  | 25                                 | Not processable                     | Evidence of static.                       |
|                                | 0.5                  | 65                                 | do                              | 0.4                  | 35                                 | V. good                             | Good.                                     |
|                                | 0.5                  | 80                                 | do                              | 0.25                 | 20                                 | do                                  | Do.                                       |
|                                | 1.0                  | 45                                 | do                              | 0.5                  | 55                                 | V. poor                             | V. good.                                  |
| Aston 108                      | 0.25                 | 80                                 | do                              | 0.5                  | 20                                 | V. good                             | Good.                                     |
|                                | 0.5                  | 65                                 | do                              | 0.5                  | 35                                 | do                                  | Fair-good.                                |
|                                | 0.5                  | 75                                 | do                              | 0.5                  | 35                                 | Good                                | Good.                                     |
|                                | 0.75                 | 65                                 | Myri 45                         | 0.5                  | 25                                 | do                                  | Excellent-good.                           |
|                                | 1.0                  | 25                                 | Nopostat LV-40                  | 0.25                 | 35                                 | do                                  | Good.                                     |
|                                | 1.5                  | 55                                 | do                              | 0.7                  | 75                                 | Not processable                     |                                           |
|                                | 1.5                  | 35                                 | do                              | 0.7                  | 45                                 | Good                                |                                           |
| Aston 123                      | 0.25                 | 80                                 | do                              | 0.25                 | 20                                 | V. good                             | Fair-good.                                |
|                                | 0.5                  | 65                                 | do                              | 0.4                  | 35                                 | Good                                | Good.                                     |
|                                | 0.5                  | 80                                 | do                              | 0.4                  | 20                                 | do                                  | Good-excellent.                           |
|                                | 1.0                  | 65                                 | do                              | 0.5                  | 35                                 | do                                  | Good.                                     |
|                                | 1.75                 | 35                                 | Syton DS                        | 0.5                  | 65                                 | Not processable                     |                                           |
| Aerotex antistatic No. 6.      | 0.5                  | 80                                 | Nopostat LV-40                  | 0.5                  | 20                                 | Good                                | Fair-good.                                |
|                                | 0.75                 | 65                                 | do                              | 0.25                 | 35                                 | do                                  | Good.                                     |
|                                | 1.5                  | 65                                 | do                              | 0.5                  | 35                                 | Fair-good.                          |                                           |

textile equipment was good or very good, and that the antistatic rating after ten machine washes was fair to good or better. It will also be noted that where the fraction of the fibers treated with the durable antistatic agent was 45% or less, the processability on textile equipment ranged from very poor down through not processable.

#### Example 3

In a similar manner, a lot of Fiber A, prepared as in Example 1, was processed on the cotton system after being properly opened. Numerous interruptions of operations for cleaning were required due to overloading of the feed roll prior to the beater in picking the fiber. The lap was poor, very soft, and uneven. Carding required use of a fancy and loading of the drum was excessive. Sliver from the card, on passing through the trumpet to the can, caused excess finish to build up in the trumpet. Drawing and roving steps were troubled with roll lapping and build-up of finish on the rolls. Spinning was troubled with finish building up on the rolls also, all causing inferior yarns to be formed.

#### Example 4

Other fibers were prepared using other permanent antistatic agents as indicated in the following table. In this table it will be seen that fibers treated with the permanent antistatic agent ranged from poor to not processable

In a similar manner, a lot of Fiber B was opened and subsequently converted to fabric with no textile processing difficulty. Picking, carding, drawing, etc. were all performed at a commercially acceptable level of performance. These fabrics, so formed, before and after being subjected to the normal predyeing scour or after dyeing had a very harsh scroopy handle characteristic of most man-made fibers. Also, after scouring or dyeing, these fibers had no antistatic protection at all.

#### Example 5

In a similar manner, a lot of Fiber B was opened and subsequently converted to fabric with no textile processing difficulty. Picking, carding, drawing, etc. were all performed at a commercially acceptable level of performance. These fabrics, so formed, before and after being subjected to the normal predyeing scour or after dyeing had a very harsh scroopy handle characteristic of most man-made fibers. Also, after scouring or dyeing, these fibers had no antistatic protection at all.

#### Example 6

Fiber C was prepared in the same manner as Fiber A (see Example 1) except that Aston 123 are used instead of Aston 108 and the product contained 1.75% durable antistatic agent based on weight of fiber.

A blend was prepared containing 33% Fiber C and 67% untreated acrylic fibers by introducing the dry fibers in the proper proportions into a wet opener and then passing the mixture through a dry opener. The resulting blend could not be processed through the cotton system under conditions approaching normal. During picking, the fibers exhibited static accumulation by adhering to the hopper walls. Also, the fibers bunched up under and behind the feed roll prior to the beater. The lap from the picker was uneven and contained many fused fibers.

Even when lighter loads of fiber were fed, successful operations were not obtained.

We claim:

1. A blend of hydrophobic synthetic fibers having improved antistatic properties and improved processability through textile machines consisting essentially of

- (a) a major proportion comprising from about 55% to about 90% of the fibers in the blend having applied thereto a durable friction-reducing antistatic agent, and
- (b) a minor proportion comprising from about 10% to about 45% of the fibers in the blend having applied thereto a ready removable friction-increasing agent.

2. A blend of hydrophobic synthetic fibers having improved antistatic properties and improved processability through textile machines consisting essentially of

- (a) a major proportion comprising from about 55% to about 90% of the fibers in the blend having applied thereto a durable friction-reducing antistatic agent, and
- (b) a minor proportion comprising from about 10% to about 45% of the fibers in the blend having applied thereto a readily removable friction-increasing antistatic agent.

3. The product of claim 2 wherein the fibers of said major proportion have applied thereto 0.25% to 2.0% of

durable friction-reducing antistatic agent on weight of fibers in said major proportion and wherein the fibers of said minor proportion have applied thereto 0.25% to 1.0% of readily removable friction-increasing antistatic agent on weight of fibers in said minor proportion.

4. The product of claim 2 wherein said hydrophobic synthetic fibers are all acrylic fibers.

5. The product of claim 2 wherein said durable friction-reducing antistatic agent comprises a product of cross-linking a linear polymer formed by the condensation of polyethylene glycol diamine and polyethylene glycol dihalide.

#### References Cited

##### UNITED STATES PATENTS

|           |         |             |             |
|-----------|---------|-------------|-------------|
| 2,832,697 | 4/1958  | Walles      | 177—138.8 X |
| 2,897,170 | 7/1959  | Gruber      | 117—139.5   |
| 2,982,751 | 5/1961  | Anthes      | 117—139.5 X |
| 3,008,215 | 11/1961 | Pitts       | 117—139.5 X |
| 3,019,132 | 1/1962  | Gabler      | 117—139.5 X |
| 3,108,011 | 10/1963 | Frotscher   | 8—115.5 X   |
| 3,167,448 | 1/1965  | Hirshfeld   | 117—139.5 X |
| 3,245,905 | 4/1966  | White et al | 117—138.8   |

WILLIAM D. MARTIN, Primary Examiner.

R. HUSACK, Assistant Examiner.